

March 19, 1940.

H. BLOUNT ET AL

**2,193,856**

## METHOD OF MAKING METALLIC RIBBON

Filed May 8, 1937

Fig. 1



Fig. 2.



Fig 3.



Fig 4



Fig 6.



Fig. 5.



Fig 7



INVENTORS  
H. BLOUNT  
H. P. ARKEMA  
CHARLES L. DUFF  
ATTORNEY

## UNITED STATES PATENT OFFICE

2,193,856

## METHOD OF MAKING METALLIC RIBBON

Harry Blount and Harold P. Arkema, Baltimore,  
Md., assignors to Western Electric Company,  
Incorporated, New York, N. Y., a corporation of  
New York

Application May 8, 1937, Serial No. 141,480

6 Claims. (Cl. 205—21)

This invention relates to a method of making metallic ribbon, and more particularly to a method of drawing such a ribbon from a round wire.

5 Heretofore it has been the practice in some instances to draw a round wire to a predetermined size and then flatten it out by passing it between a pair of rolls. On account of the high pressure per square inch on the rolls where they are 10 in contact with the wire, the rolls wear rapidly and also the grain of the metal will extend transversely of the ribbon due to the lateral expansion, which is an undesirable feature.

15 An object of the present invention is to provide an effective and efficient method for drawing a metallic ribbon of high quality.

In accordance with one embodiment of the invention a wire is selected of substantially greater cross-sectional area than a wire which is to be 20 rolled flat, and the wire is then drawn successively on two diametrically opposite sides until a ribbon of the desired thickness is obtained. A complete understanding of the invention may be had by reference to the following description, taken 25 in conjunction with the accompanying drawing, in which

Fig. 1 is a perspective view of a die and die holder;

Fig. 2 is an end view of one of the die members; 30 Fig. 3 is a side view of a die member;

Fig. 4 is a bottom view of a combined die member spacer and ribbon guide;

Fig. 5 is a longitudinal section through the die and die holder of Fig. 1, including a fragmentary view of a capstan; 35

Fig. 6 is a cross-sectional view taken on line 6—6 of Fig. 5; and

Fig. 7 is a graphic illustration of the formation of a metallic ribbon from a circular wire.

40 Referring now more particularly to the drawing, a die holder 8 is shown having a bottom portion 9 and two upright portions 11 forming substantially a U-shaped or trough-like support. The inner face of the base of the die holder is 45 provided with a pair of grooves 12, leaving a flat portion 13 upon which the die mountings 14 and 15 rest. The die mounting 14 abuts against a dowel pin 16, and its upper surface rests against a dowel pin 17. The die mounting 15 has a 50 dowel pin 18 resting against its upper surface, and the outer end of this mounting abuts against a set screw 19. After this set screw has been turned into position, it is held in position by drawing up a screw 21 which clamps the set screw 19 between the upright portions 11.

The die mountings 14 and 15 have die elements 22 with parallel surfaces secured thereto by processes well known in the art. The die elements may be made of diamonds or other suitable materials such as tungsten carbide or the like. The 5 die mountings are spaced apart a predetermined distance by means of a combined ribbon guide and spacer 23. This spacer maintains the die elements 22 a predetermined distance apart and also assists in maintaining them parallel to each 10 other. When the edges of the die elements become worn, they may be refinished and the spacer 23 is then ground down to such a length as to re-establish the desired or original spacing. The spacer has a conical aperture 26 which aids in 15 guiding the ribbon as it leaves the die elements. Fig. 5 illustrates a ribbon 24 being drawn through the die by a capstan 5. In actual practice, of course, a ribbon is formed by passing through a number of dies successively in accordance with 20 common practice in the wire drawing art.

As a specific illustration of making a metallic ribbon in accordance with the invention a typical example will be given as exemplified graphically in Fig. 7. In this figure the abscissae represent 25 area and the ordinates represent diameter or thickness.

Referring to curve A, a wire of circular cross-section having a diameter of .0158" is selected 30 representing a cross-sectional area of 100 per cent. This wire is then drawn successively through the dies until its cross-sectional area is 7.75 per cent of its original cross-sectional area. The wire is drawn successively through the dies which engage only two diametrically opposite 35 sides of the wire, and the edges of the ribbon being formed do not engage the die elements and are not drawn. It is surprising that, even though the edges of the ribbon are not drawn, and even though there is a slight increase in the width 40 of the ribbon during the drawing operations, the edges of the ribbon remain smooth and straight. When the ribbon attains a thickness of .0009", it will have a cross-sectional area of 7.75 per cent 45 of its original cross-sectional area, and the width of the ribbon will be only slightly greater than the original diameter of the wire in the specific example illustrated in curve A; the width of the ribbon after being drawn to a thickness of .0009" is .0175", which is only slightly greater than the original diameter of .0158". Since the reduction in the cross-sectional area is accomplished almost entirely by elongation, the grain of the metal will extend longitudinally of the ribbon, re- 50 55

sulting in a ribbon of high tensile strength and excellent fatigue resistance.

Curve B illustrates a method in common use in which the wire is first reduced in circular form by drawing and is then flattened by forming it between rolls. Thus, beginning with a wire of the same diameter as in the preceding illustration of .0158", the wire is drawn in circular form to .0045" in diameter, at which time it will also have 7.75 per cent of its original cross-sectional area. At this point the wire is then formed between rolls, reducing the diameter from .0045" to a thickness of .0009", in which there is practically no change in the cross-sectional area. The grain of the metal will therefore extend almost in its entirety transversely of the ribbon. A ribbon made in accordance with the invention will therefore have far superior physical properties.

It will be understood that the nature and embodiment of the invention described is merely illustrative and that many changes and modifications may be made therein without departing from the spirit and scope of the invention.

What is claimed is:

- 25 1. A method of making a metallic ribbon which comprises drawing a wire of circular cross-section through a circular die opening until its diameter is substantially equal to the width of the ribbon to be made and then drawing the wire on two diametrically opposite sides leaving the edges unrestrained to obtain the desired thickness of ribbon.
- 30 2. A method of making a metallic ribbon which comprises drawing a wire of circular cross-section through a circular die opening until its diameter is substantially equal to the width of the ribbon to be made and then continuously reducing its thickness by drawing solely on two opposite sides until a ribbon of the desired thickness is obtained.

3. A method of making a metallic ribbon which comprises drawing a wire of circular cross-section through a circular die opening until its diameter is substantially equal to the width of the ribbon to be made and then forming a ribbon substantially entirely by longitudinal deformation by reducing one diameter of said wire without changing substantially a perpendicular diameter of the wire, whereby the grain of the metal will extend longitudinally of the ribbon. 5

4. A method of making a metallic ribbon which comprises drawing a wire of circular cross section through a circular die opening until its diameter is substantially equal to the width of the ribbon to be made and then drawing the wire between die elements having straight parallel faces forming a slot substantially wider than the width of the ribbon being formed to form a ribbon having a width substantially similar to the diameter of the wire before it was drawn 10 between said parallel faces. 15

5. A method of making a metallic ribbon of a thickness of the order of .0009 inch which comprises drawing a wire of circular cross-section through a circular die opening until its diameter is of the order of .0158 inch and then drawing the wire on two diametrically opposite sides until it has the stated thickness without changing its dimension substantially along another diameter, whereby the grain of the metal will extend longitudinally of the ribbon. 20 25

6. A method of making a metallic ribbon of a thickness of the order of .0009 inch and a width of the order of .0175 inch which comprises drawing a wire of circular cross-section until its diameter is of substantially the width of the ribbon to be made and then reducing the wire along one diameter until the stated thickness is obtained. 30

HARRY BLOUNT.  
HAROLD P. ARKEMA.